

## UNITED STATES PATENT OFFICE

THEODOOR KOCH, OF ARNHEM, NETHERLANDS

PROCESS OF PREPARING ARTIFICIAL TEXTILE PRODUCTS WITH REDUCED LUSTER  
FROM VISCOSENo Drawing. Application filed October 3, 1927, Serial No. 223,831, and in the Netherlands  
February 11, 1927.

Although the high luster of artificial silk was originally considered to be one of its principal properties, for the past few years it has been proposed to bring the luster of this product in accordance with that of natural silk, and attempts have also been made to obtain a dull product which could eventually be used as a substitute for wool.

For instance the preparation of artificial silk, with a reduced luster, from viscose is already well-known. This is done by spinning immatured or only feebly matured viscose in a spinning-bath which consists of acidulated salt solutions as prevailing in nature. Another method for obtaining the same result consists of adding metal compounds to the viscose, such as calcium-hydroxide and sodium-aluminate, which cause insoluble precipitates in the thread with the constituents of the spinning-bath (sulphuric acid, monosodium-phosphate.) To obtain wool substitute with reduced luster it has already been proposed to dispense with both the ripenings and to spin immediately after zanthogenization in a spinning bath of a dilute mineral acid.

Besides some drawbacks met with in the technical application, these processes have a further disadvantage that the products obtained in this way may hardly take the name of artificial silk, especially with regard to the feeling, tensile strength and elongation.

In contradistinction herewith, the new products according to my invention, have the advantage that in view of feeling, drying and other properties, they may be compared with ordinary artificial silk or may be even better quality, not having the very dazzling luster of ordinary artificial silk, but more the quiet luster of natural silk. According to my invention however, it is also possible to obtain entirely dull products without any luster whatever, if for any reasons, they may be required.

The new composition of matter according to my invention comprises viscose containing chlorobenzene or a mixture of mono- and dichlorobenzene.

By the term "immiscible" is intended those substances which can only be incorporated

in a state of fine division in the viscose to form an emulsion by intense agitation as distinct from substances which are normally soluble in the viscose or readily form a colloidal solution therein.

In order to obtain a product of the desired properties, it is of considerable importance that the additions are very finely mixed with the viscose. This is obtained if, for instance, according to my invention, additions or mixtures of additions are used, the specific weight of which must correspond practically with that of the viscose to be worked up.

## Example 1

To normal viscose one per cent of mono-chlorobenzene is added and this substance is divided very finely in the spinning liquid by intensified agitation. The viscose thus prepared is spun in the usual way at a ripeness of about 9.5 Hottenroth at about 40°-45° C. in a spinning bath containing 12% of magnesium sulphate, 12% sodium-sulphate, and 10% sulphuric acid. Thereupon is the product finished, and the addition evaporates on drying the spun material. A thread of good physical properties is obtained, possessing, however, a reduced luster.

The amount of the reduction of luster depends upon the proportion of the addition.

## Example 2

One per cent. of a mixture of mono- and dichloro-benzene of a specific weight corresponding with that of the viscose of 1.12 is added and thereupon emulsified. At the usual ripening temperature no separation of the mixture takes place, and also no separation after a week notwithstanding the usual intermediate filtrations.

The spinning liquid is spun at the ripeness and in a spinning bath as described in Example 1, whereupon the silk is finished and dried in the normal way. A product is obtained of very much reduced luster of good elongation and tensile strength.

## I claim:

1. As a new composition of matter to be spun into artificial silk, viscose containing chlorobenzene.

2. As a new composition of matter to be spun into artificial silk, viscose containing a mixture of mono- and di-chlorobenzene.

3. As a new composition of matter to be spun into artificial silk, viscose to which has been added a mixture of mono- and di-chlorobenzene in such relative proportions that the specific weight of the addition is practically in accordance with that of the viscose to be

10 worked up.

4. As a new composition of matter to be spun into artificial silk, viscose to which has been added approximately 1% of a mixture of mono- and di-chlorobenzene in such relative proportions that the specific weight of the addition is practically in accordance with that of the viscose to be worked up.

In testimony whereof I affix my signature.  
THEODOOR KOCH.

20

25

30

35

40

45

50

55

60

65